

## UNITED STATES PATENT OFFICE

2,165,441

## FREE-CUTTING ALUMINUM ALLOYS

Adolf Beck and Hans Bohner, Bitterfeld, Germany, assignors to I. G. Farbenindustrie Aktiengesellschaft, Frankfort-on-the-Main, Germany

No Drawing. Application June 19, 1937, Serial No. 149,207. In Germany June 25, 1936

5 Claims. (Cl. 148—21.1)

This invention relates to a process of rendering aluminum alloys suitable for working with cutting tools.

Aluminum alloys have been proposed which 5 contain, besides at least 3% of magnesium, additions (to a total extent of 1 to 5%) of one or more alloying components such as manganese, chromium, iron, titanium, vanadium, tungsten, cobalt and nickel which form, with the aluminum, hard and brittle inter-metallic compounds which are practically insoluble in the aluminum.

Further investigations have now shown that 15 these aluminides primarily crystallising out of the molten alloy, occur mainly as large crystals, especially when the additions consist of manganese, chromium or iron, singly or in conjunction. It has been found that if such alloys be worked with cutting tools, particularly at high 20 speeds, these crystals are easily torn out of the structure by the tool steel, so that the worked surface is roughened.

It has now been ascertained, in accordance 25 with the present invention, that a heat treatment (hereinafter referred to as "disintegrating heat treatment") at temperatures above 300° C. and the eutectic temperature of the alloy (450° C.), causes the 30 large primary crystals of hard, inter-metallic aluminides, by interaction with the surrounding aluminum-magnesium solid solution, or with the aluminum-magnesium compounds separating out during solidification, to break up into a number 35 of smaller crystals. By this means, the formation of a rough surface during the working of the alloy with high speed cutting tools, is avoided.

In many instances it has also been found 40 advantageous to apply, before or after the disintegrating heat treatment for breaking down the primary crystals, a further heat treatment (hereinafter referred to as "heterogenising heat treatment") leading to a segregation in the matrix of the alloys, of components previously present in supersaturated solid solution, since the presence 45 of the finely divided segregate facilitates the breaking down of the large, primarily separated aluminides into numerous small crystals. Obviously however the application of such heterogenising heat treatment presupposes the alloy 50 to be in a state in which at least part of the  $Al_3Mg_2$  compound is held in supersaturated solution, i. e. is of a more or less homogeneous texture.

In order to produce such heterogenisation, the 55 alloy is subjected, in known manner, to an an-

nealing treatment at temperatures below the boundary line between the  $\alpha$  and the  $\alpha+\beta$  fields in the phase diagram of the binary aluminum-magnesium alloys, but, on the other hand, sufficiently high, i. e. at least about 200° C., and preferably within a temperature range extending from the said boundary line to about 50° C. below said line, to produce extensive heterogenisation of the supersaturated mixed crystals owing to the segregation of the compound  $Al_3Mg_2$ . The same result 10 is known to be obtainable by suitably retarding the cooling of the alloy from the temperature range in which it is, according to the phase diagram, homogeneous.

The disintegrating and heterogenising heat 15 treatments above referred to can be applied in direct succession. In the case of alloys of a magnesium content exceeding about 6%, in which heterogenisation may be effected by the application of temperatures exceeding about 300° C., the 20 disintegrating heat treatment may even be combined with the heterogenising heat treatment, since the application of one and the same temperature between about 300° C. and the boundary line separating the  $\alpha$ — from the  $\alpha+\beta$  field will 25 produce both effects simultaneously.

If an alloy, which has undergone the disintegrating heat treatment—and in which therefore the primary aluminide crystals are already 30 present in a broken-down condition—be subjected to plastic deformation, this operation will result in an extensive distribution of the disintegrated crystals of the primary aluminides, so that, after 35 deformation, numerous small aluminide crystals are present, in a more or less uniform condition of distribution, in the structure of the alloy. When such alloys are worked with cutting tools, the worked areas exhibit a perfectly smooth surface.

Owing to the improved distribution, in the 40 structure of the alloy, of the crystals facilitating the formation of cuttings, as the result of the disintegrating heat treatment of the present invention, it is possible substantially to reduce the amounts of metals, added for the purpose of 45 forming hard, intermetallic compounds, by comparison with those hitherto considered necessary, additions of not less than 0.5% and not more than 3% being sufficient. By this means, substantial advantages are gained, both in the melt- 50 ing process and in all the subsequent treatments.

The alloys may also contain up to 10% of one or more of the elements zinc, silicon and copper, which are absorbed, in the form of a solid solution, into the matrix or, in some cases, also 55

separate from the matrix as binary compounds with the magnesium, or also as more complex compounds.

*Example I*

5 An aluminum base alloy containing 9% of magnesium and 1.5% of chromium obtained on cooling from the molten state is subjected to a disintegrating heat treatment at a temperature from 400 to 450° C. and then pressed. The structure reveals numerous small crystals uniformly distributed throughout the matrix.

*Example II*

15 A structure similar to that described in Example 1 is obtained when an aluminum base alloy containing 9.5% of magnesium, 0.6% of chromium and 0.2% of manganese after casting, solidification and cooling, is annealed for 10 hours at 270 to 300° C. and thereupon subjected to a disintegrating heat treatment for 5 hours at a temperature of from 400 to 420° C., and subsequently extruded. In order still further to disintegrate the primary crystals the alloy after being extruded, is subjected to a further heterogenising heat treatment for 1 hour at a temperature of 300° C.

*Example III*

30 An aluminum base alloy containing 10% of magnesium, 0.2% of titanium, 0.35% of chromium and 0.5% of silicon is subjected to a heat treatment according to either Example I or Example II, and furnished a similar structure favourable for working with cutting tools.

We claim:

1. Process of improving the properties in re-

spect of working with cutting tools, of aluminum base alloys containing besides at least about 3% of magnesium a total quantity of from about 1 to about 5% of at least one metal forming hard intermetallic compounds with aluminum and adapted to react peritectically with the aluminum-magnesium compound formed in such alloys, which process comprises subjecting such alloy in the solid state to a heat-treatment within the temperature range extending from about 300° C. upwards, until disintegration of the primary crystals of the hard intermetallic compounds has taken place.

2. Process in accordance with claim 1 as applied to alloys containing more than about 6% of magnesium, in which the disintegration treatment is carried out at temperatures below the boundary line separating the  $\alpha$ - and the  $\alpha+\beta$  field of the aluminum-magnesium alloy phase diagram and is preceded by a homogenising treatment.

3. Process in accordance with claim 1 as applied to alloys containing magnesium in the form of a super-saturated solid solution, in which the disintegrating heat treatment is combined, in the form of a separate step, with a heat-treatment adapted to cause segregation of at least part of the magnesium held in supersaturated solution.

4. Process in accordance to claim 1, in which the disintegrating heat treatment is followed by a plastic deformation.

5. A process in accordance with claim 1, in which the disintegrating heat-treatment is carried out at temperatures between about 400° C. and 450° C.

35  
ADOLF BECK,  
HANS BOHNER.